

# UNITED STATES PATENT OFFICE.

EDWIN TATHAM, OF BALMAIN, NEAR SYDNEY, NEW SOUTH WALES.

## METHOD OF MAKING GAS.

SPECIFICATION forming part of Letters Patent No. 499,483, dated June 13, 1893.

Application filed September 10, 1889. Serial No. 323,533. (No model.)

*To all whom it may concern:*

Be it known that I, EDWIN TATHAM, gas-engineer, a subject of the Queen of Great Britain, residing at No. 76 Mullens Street, Balmain, near Sydney, in the Colony of New South Wales, have invented a certain new and useful Improvement in an Improved Gas, usable as an explosive and in admixture with other gases as an illuminating and heating gas; and

10 I do hereby declare that the following is a full, clear, and exact description of the invention, which will enable others skilled in the art to which it appertains to make and use the same.

15 The object of this invention is the production of a gas the principal uses of which are as a motive power in gas and explosive engines, as a destructive force for blasting and like purposes, but which may also be used in 20 admixture with other gases, for instance to intensify or bring out their illuminating power. This gas made according to my process is comparatively cheap in cost, is comparatively safe to handle, and yet when ignited has a highly explosive force.

25 My invention consists essentially in combining oxygen or commercially pure oxygen (such for instance as that made by the so-called Brin process and which contains only 30 about five per cent. of nitrogen) with hydrocarbon, so as to form an explosive compound. The oxygen is drawn or forced through or over liquid hydro-carbon, as for instance benzine, crude oil, gasoline, kerosene, naphtha, or 35 such like in a mixing vessel in which the hydrocarbon and the oxygen commingle, the latter combining in its due or suitable proportion with hydrocarbon so as to form a gaseous compound of a comparatively fixed or permanent character, because, as I have discovered, 40 oxygen has a far greater carrying power for hydrocarbon vapors than other gases have. This gas, so made, can then be drawn off for

use. If a hydrocarbon of great density is used I heat it before the oxygen is passed through it. When hydrocarbons such as spirits or light oils of a density of about 725° on Sykes' hydrometer are used, I find the ordinary temperature of about 60° Fahrenheit to be sufficient, but when hydrocarbons such as heavy oils of a density of about 900° by Sykes' hydrometer are used I heat the same to about 212° Fahrenheit which may be done by providing the reservoir with a steam jacket; or vice versa, I heat the oxygen to about 200° or 300° Fahrenheit before passing it into the reservoir.

45 I would have it understood that I do not confine myself to any precise manner of or means for manufacturing my explosive gas, so long as the nature of my invention be retained. It must also be distinctly understood that in my explosive gas the percentage of hydrocarbon must never exceed forty by volume, and that usually and advantageously it 55 would vary between four per cent. and twenty per cent.

Having thus described my invention, what I claim is—

1. The method of manufacturing explosive gaseous compounds, which consists in combining oxygen containing but a small proportion (about five per cent.) of nitrogen, with a hydrocarbon gas in a proportion not exceeding forty per cent. of the oxygen per volume, as 75 set forth.

2. An explosive gaseous compound or mixture, consisting of hydrogen, carbon, and pure or substantially pure oxygen in about the proportions set forth.

Dated this 18th day of July, 1889.

EDWIN TATHAM.

Witnesses:

FRED WALSH,  
F. M. Inst., P. A.  
THOS. J. WARD.